

1

3,374,157  
**ELECTROLYTE FOR THE ELECTRODEPOSITION  
 OF TECHNETIUM**  
 Willard D. Box, Oak Ridge, Tenn., assignor to the United  
 States of America as represented by the Secretary of the  
 United States Atomic Energy Commission  
 No Drawing. Filed May 21, 1965, Ser. No. 457,872  
 2 Claims. (Cl. 204—45)

The present invention relates to a method and composition which permits quantitative electrodeposition of Tc from an aqueous solution of sulfuric acid.

Technetium-99 is a low energy beta emitter, with a simple decay scheme, decaying to the stable ruthenium-99 isotope. Among other areas of utility the soft beta (0.29 mev.) rays of Tc-99 can be used to hasten blood coagulation in eye surgery to minimize scar formation. Other areas of utility are as beta calibration sources and as static eliminators. To be useful for any of these or similar purposes, it is usually necessary to provide the Tc as a thin-layered adherent deposit on a metallic substrate. It is also preferable that the Tc deposit be of high purity and the yield of Tc metal as deposited from a given plating solution be high. By high yield, I mean that in excess of 99% of the Tc in solution can be electrodeposited as a thin, smooth, adherent layer on a cathode surface within a reasonably short time.

The present invention meets this objective by providing for the electrodeposition of Tc from an electroplating solution comprising an aqueous solution of sulfuric acid containing dissolved technetium, as pertechnetate ion, and a polycarboxylic acid selected from oxalic acid, citric acid, tartaric acid, glutaric, malonic, succinic, and ammonium salts thereof.

Electroplating of technetium from a pertechnetate solution of sulfuric acid is known. Thus, for example, J. D. Eakins and D. G. Humphries have reported in the *Journal of Inorganic Nuclear Chemistry*, vol. 25 (6) :737 (1963) the electrolytic deposition of Tc from a solution of ammonium pertechnetate in 2 M sulfuric acid. It was found that deposition of technetium was terminated after only a quarter of the total technetium in solution had been deposited, with the remainder having been converted to an insoluble form.

In accordance with the present invention an electrolytic bath is provided from which technetium can be electrodeposited with virtually total yield efficiency as a smooth, adherent deposit on the surface of a selected metal substrate. The improved electrolytic bath comprises an aqueous solution of sulfuric acid containing pertechnetate as ammonium pertechnetate and a pertechnetate stabilizing agent selected from oxalic acid, citric acid, tartaric acid, glutaric, malonic, succinic, and ammonium salts thereof. I use the term "technetium stabilizing agent" in the sense that the oxalate or other polycarboxylic acid of the defined class apparently retains the technetium in pertechnetate form and prevents reduction to lower valence states as evidenced by precipitate formation.

The preparation of the electrolytic bath is effected by dissolving ammonium pertechnetate in an aqueous solution of the free acid or in the ammonium salt form of the selected pertechnetate stabilizing agent. A preferred solution is ammonium pertechnetate dissolved in at least 0.4 M ammonium oxalate to which sufficient sulfuric acid is added to reach a solution pH in the range 1 to 2. The hydrogen ion concentration in solution in combination with the material used as cathode, will determine whether the technetium plates are used as metal or as an oxide.

By placing the aforementioned technetium solution in a tank such as a glass vessel containing a platinum gauze anode facing a selected metal foil or sheet as cathode, and joining the cathode and anode through an external DC

2

power supply, electroplating of Tc as metal or oxide can be effected. I have found that a 0-20 volt, 0-20 amp. 400 watt DC source will furnish sufficient current to effect electrodeposition.

The following examples will illustrate the efficiency of the novel electroplating bath, as well as pointing out the operational and preferred parameters.

#### Example I

In this example Tc was electrodeplated from 3 separate solutions each consisting of 150 ml. of a solution of ammonium pertechnetate containing 0.7 M oxalate, each of said solutions being adjusted to 0.45 in sulfuric acid. A copper cathode and a platinum gauze anode was used in electroplating the Tc. The copper cathode was weighed before and after Tc deposition. Plating was effected at room temperature (25° C.) using a cathode current density in the range 1.0 to 1.3 amp./cm.<sup>2</sup> to produce a smooth adherent deposit. Higher deposition rates or higher plating temperatures tend to produce less adherent deposits. The electrolysis was continued until no further weight gain was detected on the cathode. The weight of the Tc dissolved in the solution, the amount of Tc deposited and the percent yield is listed below in Table I.

TABLE I

| Run No. | Te in Electrolyte, mg. | Te deposited, mg. | Yield, Percent |
|---------|------------------------|-------------------|----------------|
| 1-----  | 25                     | 24.86             | 99.5           |
| 2-----  | 9.81                   | 9.73              | 99.2           |
| 3-----  | 6.56                   | 6.53              | 99.6           |

It will be seen that in each run substantially all of the technetium in solution was deposited on the cathode. By contrast, the technetium deposition yield efficiency from solutions which did not contain the technetium stabilizing oxalate reagent reached a value of about 25%, whereupon the dissolved technetium precipitated and further deposition ceased. Examination of any of the metallic deposits under a high-power microscope showed the technetium metal deposited on the cathode surface as microscopic spheres (ranging from 0.00008 to 0.00007 inch in diameter) built up in layers. By wiping the surface of the deposit with light tissue paper several times any loose technetium can be removed so that a background reading of less than 10 disintegrations per minute is reached in the third to fifth wiping. The technetium surfaced element is then ready for use for any of the aforementioned or similar purposes.

#### Example II

This example illustrates the purity of Tc deposit attainable by the present invention.

From a solution containing 10.27 mg. sample of technetium, plating was effected on a metal (platinum) cathode in accordance with the procedure of Example I. The deposited technetium was dissolved in an ammonium hydroxide solution containing H<sub>2</sub>O<sub>2</sub>. The resultant solution was split into two aliquot portions. A coulometric analysis showed a total of 10.19 mg. technetium in solution while a polarographic analysis showed 10.16 milligrams—thus representing a Tc purity of 99%.

#### Example III

This example shows how process parameters may be varied to yield a technetium metal or oxide deposit, as desired.

According to this invention, technetium may be plated as metal or oxide depending on the concentration of technetium stabilizing reagent and sulfuric acid in solution. For example, using a fixed amount (0.7 M) oxalate as the technetium stabilizing reagent and a copper cathode, the minimum acid concentration was 0.45 M; with platinum as the cathode the minimum acid concentration

necessary to obtain a Tc metal deposit was 1.90 M. The various metals used as cathodes and the acid concentrations for metal and oxide deposition are listed in Table II below using a constant oxalate concentration of 0.7 M.

TABLE II

| Cathode              | H <sub>2</sub> SO <sub>4</sub> Concentration, molar |           |
|----------------------|-----------------------------------------------------|-----------|
|                      | For Metal                                           | For Oxide |
| Copper.....          | 0.45                                                | 0.32      |
| Nickel.....          | 0.87                                                | 0.58      |
| Aluminum.....        | 1.14                                                | 0.71      |
| Silver.....          | 1.41                                                | 0.87      |
| Gold.....            | 1.41                                                | 0.87      |
| Stainless Steel..... | 1.41                                                | 0.87      |
| Platinum.....        | 1.90                                                | 1.14      |

The oxalate concentration necessary in the electrolyte for the Tc metal or oxide deposition depends on the acid concentration in solution. For example, when copper is the cathode and electrodeposition is effected from a solution 0.4 M in oxalate, an acid concentration of 1.90 M will yield a technetium oxide deposit. When the oxalate concentration is increased to 0.7 M a technetium metal deposit with an acid concentration of only 0.45 M is formed. As a matter of convenient operation, I prefer to use a saturated solution of the technetium stabilizing reagent, while varying the acid concentration according to whether a metal or oxide deposit is desired.

It will be seen that I have described a novel electroplating bath for use in the efficient electrodeposition of technetium to form a smooth, adherent deposit on a metal substrate. The invention has been described and illustrated in use with an oxalate salt as the technetium stabi-

lizing reagent. However, it should be understood that the same general order of plating efficiency will be realized when practicing the invention with the class of polycarboxylic acids and ammonium salts previously defined.

Having thus described my invention, I claim:

- An electrolytic plating bath for technetium comprising an aqueous solution of sulfuric acid containing technetium as pertechnetate ion, and a stabilizing amount of a polycarboxylic acid selected from the group consisting of oxalic, glutaric, malonic, succinic, tartaric, and citric acids and ammonium salts thereof, sufficient to prevent reduction of the pertechnetate in solution to a lower oxidation state, said bath having a pH in the range of 1 to 2.

2. The electrolytic plating bath recited in claim 1 in which the pertechnetate stabilizing reagent is ammonium oxalate.

## References Cited

## UNITED STATES PATENTS

2,497,725 2/1950 Griffith 204—105

## OTHER REFERENCES

Journal of Inorganic and Nuclear Chemistry, vol. 25, No. 6, pp. 737—739, June 1963.

Radioisotopes, vol. 8, No. 1, pp. 32—33, March 1959.

The Journal of Chemical Physics, vol. 13, No. 6, pp. 269—276, July 1945.

30 HOWARD S. WILLIAMS, Primary Examiner.

G. KAPLAN, Assistant Examiner.